

## UNITED STATES PATENT OFFICE.

FREDERICK CARL NIEDERHAUSER AND HAYDEN BENJAMIN KLINE, OF CLEVELAND,  
OHIO, ASSIGNORS TO THE INDUSTRIAL RAYON CORPORATION, OF CLEVELAND,  
OHIO.

## PROCESS FOR TREATING CELLULOSIC MATERIAL.

No Drawing.

Application filed December 18, 1926. Serial No. 155,763.

This invention relates to the application and use of relatively small amounts of combinations of the alkali metals with zinc, of which the alkali metal zincates are perhaps 5 the best known, in the rayon artificial filament art, and to methods for producing rayon wherein combinations of alkali metal and zinc or alkali metal zincates are employed in order to produce in the finished 10 rayon material desirable properties as will be more specifically detailed in this specification. These alkali-zinc compounds are rather loosely characterized chemical bodies, and may be formed by dissolving metallic 15 zinc, zinc oxide, zinc hydroxide or other zinc compound, or water-soluble zinc salts such as zinc chloride, zinc nitrate or zinc sulfate in solutions of the alkali metal hydroxides to form the zincate desired. These 20 zincates or solution of zinc in alkali metal hydroxide are introduced in amounts stated in our process at stages in the manufacture of viscose rayon, prior to the formation of the viscose into filaments, that is, before 25 the xanthated cellulose has been projected thru the spinnerets into the coagulating or precipitating bath. The method or details of forming alkali metal zinc compounds or alkali metal zincates comprise no portion of 30 our process as disclosed in this specification.

More specifically, our process is concerned with the introduction into the process for viscose manufacture of relatively small amounts of alkali zincate, and inasmuch as 35 sodium hydroxide is the alkali metal hydroxide used for the treatment of cellulose in present day viscose manufacture, the description herein will be limited to the application of sodium zincate, we having found 40 that other alkali metal zincates may be used in our process such as potassium zincate or ammonium zincate with satisfactory results. The sodium zincate may be prepared by the addition of the calculated amount of zinc salt—preferably a water-soluble zinc salt 45 for greater ease in manipulation—directly to the sodium hydroxide when the latter is being dissolved in water to form the concentrated or stock solution from which the 50 sodium hydroxide solution is prepared that is used to treat the cellulosic material; or the sodium zincate may be added to this stand-

ard sodium hydroxide solution after the same has been adjusted as to concentration to the degree desired for alkali-cellulose formation with the cellulosic material used; or the alkali metal zincate in alkali metal hydroxide solution in water may be sprayed or otherwise incorporated with the alkalinized cellulose during the disintegration of the 55 same in the mixer or Pfeiderer; or the sodium zincate may be added to the xanthating churn during, prior or subsequent to the addition of carbon bisulfide to the alkalinized cellulose; or the sodium zincate solution may be incorporated with the sodium hydroxide solution used to thin or dilute the xanthated cellulose preparatory to submitting the same to the xanthate ripening or maturing process; or it may be added to the partially ripened or immature viscose solution. We have 60 obtained satisfactory results by adding the sodium zincate to each of the stages above mentioned, but find it more convenient to form sodium zincate by the addition of the 65 required amount of water-soluble zinc salt such as zinc sulfate, directly to the sodium hydroxide in the formation of the initial solution of the same, and hence the zincate is present at each stage of the process prior 70 to the actual spinning operation. It will be evident, that adjustment as to the percentage of zincate incorporated will be made 75 dependent upon whether the zincate is added before or after the process of mercerization or alkali-cellulose formation wherein a portion of the zincate is removed with the excess of sodium hydroxide solution used, or whether the zincate is added in a step in the process in which no portion of it is removed 80 by a subsequent step in the normal operation of viscose manufacture. We have added the water soluble zinc salt to the cellulosic material before the latter has been run into the sheet form, but find this is not the most convenient step in the process of viscose manufacture to introduce the zinc. 85

The process of viscose manufacture is not materially accelerated, inhibited or otherwise changed as the result of the addition thereto and therein of the amounts of zincate employed by us, in so far as we have been able to determine. In reality, our research has shown that the addition of the 90 95 100

soluble zinc in the process of viscose manufacture, before the finely divided alkali cellulose has been matured, has a tendency to shorten the time of maturing. We have also 5 found this tendency when the comminuted alkalized cellulose has been ripened in cans made of zinc, and the contents of the cans have been periodically mixed, in order to bring new alkali-cellulose surfaces in contact with the zinc in the presence of free alkali metal hydroxide. One object of the 10 addition of alkali metal zincate in the otherwise normal process of viscose manufacture, is to produce a rayon filament of enhanced luster, additional covering power, increased 15 fluffiness, and usually a whiter bleached rayon is obtained, than when the process of rayon viscose manufacture is conducted without the introduction of the zincate. Photo- 20 micrographic variations between filaments treated by alkali metal zincates; and a filament not so treated are evident.

It is apparently immaterial whether the 25 water-soluble zinc salt be a chloride, nitrate or sulfate, the relatively small amount of acid radical present after zincate formation, exercising no noticeable effect upon the process or the result obtained. It is also immaterial whether the sodium zincate be prepared 30 as such and introduced into the process of viscose manufacture at the step desired, or whether the zincate be formed in the alkali hydroxide solution employed to mercerize the cellulose or to dilute and attenuate the xanthated cellulose. In any event, 35 the introduction of zincate is made prior to the ripening of the viscose to the phase desired for optimum spinning purposes.

In the incorporation of the desired amount 40 of zincate, it has been found advantageous to add the water-soluble zinc salt such as zinc sulfate in crystal form directly to the caustic soda dissolver, in forming the concentrated stock solution in order that the formation 45 of the sodium zincate may be accelerated, and the formation of zinc hydroxide minimized or prevented, due to the higher temperature and concentration of the caustic in the initial dissolving process. We 50 have obtained satisfactory results in viscose rayon manufacture when the sodium zincate was present in the mercerizing or steep liquor to the extent of 0.04% to 1.5% but it is to be understood that the percentages 55 above stated may be varied in some adjustments of the process without departing from the spirit or essence of our invention. If the zincate is added at any stage of the process subsequent to alkali-cellulose formation and expulsion of excess alkali from the alkali-cellulose formed, a correspondingly lesser amount will be required, as will be understood by those skilled in the art. We 60 have obtained excellent results over a considerable period of experimentation when

the sodium zincate percentage in the steep bath was maintained between the limits of 0.05% to 0.1%.

If the zinc is to be added to the dissolving sodium hydroxide which is used for the final solution of the xanthate, the alkali zinc compound should have been previously prepared due to the fact that zinc sulfate when introduced into weak caustic solutions, favors the formation of zinc hydroxide rather than alkali zincates. That is, the alkali metal hydroxide concentration must be sufficient to dissolve zinc hydroxide. From the viewpoint of factory expediency, we do not find it preferable to introduce the zincate-compound into the Pfeiderer during the process of mastication of the alkali cellulose, or in the xanthate drum during the process of viscose formation.

As an example of carrying our process into effect, we may add to the caustic soda solution being dissolved for stock solution to be afterwards used for mercerization of cellulosic material, an amount of zinc chloride so that the percentage of sodium zincate in the sodium hydroxide solution 0.05-0.1%, plus or minus one-hundredth of one percent, the process being then carried on identical as if the zinc compound had not been present. The viscose rayon produced had an appreciably increased covering power and fluffiness, had a whiter color when submitted to the normal bleaching process, and under the microscope the cross section of individual filaments had to a notable degree the desirable serrated appearance.

Having now described our invention and in what manner it may be carried into effect, what we claim and desire to secure by Letters Patent is:—

1. In a process for the manufacture of viscose rayon, the introduction in an alkaline medium into the process of viscose manufacture of an alkali metal zincate in solution, said zincate being incorporated into the alkaline viscose solution prior to the maturing of the viscose to the stage desired for precipitation, the solution being afterwards forced through openings into a precipitating bath for the formation of filaments, as herein set forth.

2. In a process for the manufacture of viscose rayon, the introduction in an alkaline medium into the process of viscose manufacture of an alkali metal zinc compound in solution in amount insufficient to cause precipitation of the viscose and prior to the maturing the viscose to the stage of precipitation, the solution being afterwards forced through openings into a setting bath for filament formation, as herein set forth.

3. In a process for the manufacture of viscose rayon, the introduction into an alkaline medium into the process of viscose manufacture of an alkali metal zinc com-

pound in solution, said alkali metal zinc compound being incorporated prior to the maturing of the viscose solution to the stage where filaments may be formed, as herein set forth.

4. In a process for the manufacture of filaments of viscose the introduction in an alkaline medium into the process of viscose manufacture, of sodium zincate in amount insufficient to cause precipitation of the viscose in solution, said sodium zincate being added at any stage of the process prior to the maturing of the viscose to the stage best suited for spinning purposes, said solution being afterwards forced into a precipitating medium, substantially as herein described.

5. In the usual process for the manufacture of viscose intended for the formation of filaments and films, the addition to the caustic soda employed, of alkali metal zincate in amount equivalent to not less than 0.04% of the cellulosic material originally used, substantially as described herein.

6. A process for the manufacture of viscose comprising the usual steps of steeping, disintegrating and mixing, maturing, xanthating, diluting with sodium hydroxide and maturing the diluted xanthate, but in which a portion of the sodium hydroxide normally employed is replaced by a sodium hydroxide solution of sodium zincate in amount equivalent to not less than 0.04% of the cellulose originally employed, as set forth herein.

7. A process for the manufacture of xanthated cellulose comprising dissolving an alkali metal zincate in alkali metal hydroxide and using said alkali metal hydroxide in the steps normally necessary to produce viscose for filament and film formation, as detailed herein.

8. A process for the manufacture of xanthated cellulose, comprising steeping, disintegrating and mixing, maturing, xanthat-

ing, diluting and ripening in the usual manner except that instead of the employment of sodium hydroxide, there is used a sodium hydroxide-containing sodium zincate dissolved therein, the amount of sodium zincate used being from 0.04% to 1.5% on the weight of the cellulose originally used, substantially as set forth herein.

9. In a process for the normal manufacture of viscose suitable for rayon formation, the substitution for sodium hydroxide solution, of an amount of sodium hydroxide solution containing an amount of zinc dissolved therein insufficient to cause precipitation of the viscose, afterwards forcing the solution containing viscose and zinc compound into a precipitating bath through orifices, substantially as set forth herein.

10. A process for the manufacture of viscose suitable for rayon production, consisting in steeping cellulosic material in sodium hydroxide solution of 18.8% strength and containing dissolved therein sodium zincate in amount from 0.04% to 1.5%, then disintegrating and mixing, maturing, xanthating, thinning with caustic soda solution and maturing in ways now known, as set forth herein.

11. In a process for the manufacture of viscose products from cellulosic materials, carrying out the usual steps of viscose manufacture up to the point of precipitation of the ripened viscose, but substituting for a portion of the sodium hydroxide used in the steps preceding the precipitation of the matured viscose, sodium hydroxide, containing an amount of alkali zincate equivalent to 0.04%-1.5% by weight of the original cellulosic material employed, as described herein.

In testimony whereof we affix our signatures.

FRED. C. NIEDERHAUSER.  
HAYDEN B. KLINE.